

## UNITED STATES PATENT OFFICE

FREDRICH OLSEN, OF DOVER, NEW JERSEY

## DELAY POWDER

No Drawing.

Application filed October 30, 1928. Serial No. 671,751.

The subject matter of the present invention is a delay powder.

The primary object of this invention is the provision of a slow burning composition especially adapted for use as a delay.

With the foregoing and other objects in view, my invention resides in the novel arrangement and combination of ingredients hereinafter described and claimed, it being understood that changes in the precise embodiment of the invention herein disclosed may be made within the scope of what is claimed without departing from the spirit of the invention.

Heretofore, black powder has most generally been used as a delay element in fuses, propellants, and indeed wherever a delay is desired. While in many ways suited for this purpose, because of its cheapness and ease of preparation ordinary black powder has certain disadvantages, the principal one of which, at the present time, is the impossibility of regulating the rate of burning. I have found, however, that if the proportions of the ingredients in black powder or a powder having a similar composition are modified so as to permit the addition of a deterrent, the desired rate of burning may be attained while at the same time the resultant composition will answer all the purposes of a delay.

The powder which forms the subject of my invention may be made directly by varying the proportions of the black powder ingredients so as to permit the addition of the necessary amount of a deterrent agent or by mixing sulphur, charcoal and any equivalent of potassium nitrate with the necessary amount of deterrent.

A composition which has proved successful in practice is as follows:

|                    | Per cent |
|--------------------|----------|
| Charcoal           | 15.3     |
| Sulphur            | 8.4      |
| Potassium nitrate  | 74.1     |
| Triphenylphosphate | 2.2      |

While the composition cited in the formula given has met all requirements, I do not propose to limit my invention to the proportions or ingredients used. For potassium nitrate

any other suitable oxidizing agent such as sodium nitrate or barium nitrate may be substituted, and instead of the triphenylphosphate any other suitable deterrent may be employed such as camphor, dimethylphenyl orthotolylurea, diphenyl dimethylurea, dinitrotoluene or petrolatum. The quality of the charcoal may also be varied from hard burned to soft burned and the source of this charcoal may be willow, alder, weeds, etc.

It has been found further that by changing the percentage of the deterrent, in the composition that the rate of burning may be altered.

A powder made according to the formula outlined or having any similar composition, may be made by any well known method of making black powder.

A delay composition made according to my invention has been found especially useful as a delay element in fuses, though, by no means limited to this use.

I claim:

1. A slow burning powder composition including approximately 15.3% charcoal, 8.4% sulphur, 74.1% potassium nitrate, and 2.2% triphenylphosphate.

2. A slow burning powder composition including charcoal, sulphur, potassium nitrate, and triphenylphosphate.

3. A slow burning powder composition including charcoal, sulphur, a nitrate of an alkali earth metal and triphenylphosphate.

4. A slow burning powder composition including charcoal, sulphur, a nitrate and triphenylphosphate.

5. A slow burning powder composition including charcoal, sulphur, an oxidizing agent and triphenylphosphate.

FREDRICH OLSEN.

90

95

100